

## 1

3,384,501

### STEARATO CHROMIC CHLORIDE PRINTING PROCESS

James S. Crump, Mobile, Ala., assignor to International Paper Company, New York, N.Y., a corporation of New York  
No Drawing. Continuation of application Ser. No. 405,844, Oct. 22, 1964. This application June 26, 1967, Ser. No. 649,052  
2 Claims. (Cl. 106—287)

#### ABSTRACT OF THE DISCLOSURE

A process of printing a stearato chromic chloride formulation at spaced intervals on wrapping paper by means of a printing press for the purpose of having such formulation serve as an adhesive releasing agent where printed.

This application is a continuation of application S.N. 405,844 filed Oct. 22, 1964, now abandoned.

This invention relates to a novel adhesive releasing agent. More particularly, it relates to a method for providing an adhesive releasing surface on wrapping paper or any other material otherwise subjected to contact with an adhesive.

Recently, a major producer of shingles for roofing and the like has been making such shingles with a strip of a new type of resinous adhesive along the top side of each shingle. This strip of adhesive serves as a means by which the overlapping shingles seal themselves together under the influence of the sun's heat and their own weight.

As might be expected, the presence of the strip of adhesive on each shingle posed a packaging problem. Since the packaged shingles were necessarily exposed to a certain amount of heat and pressure in storage, it transpired that the top shingle in each package of twelve stuck to the packaging, i.e., kraft wrapping paper, and was thereby made useless as a roofing material.

In an attempt to overcome the problem of the sticky shingles, the shingle producer developed a method of applying a latex emulsion to the wrappers for each set of twelve shingles as each wrapper was used on a shingle wrapping machine. But it was found that neither the emulsion nor the machine achieved reliable or consistent results.

In the development of the present invention, it was found that not only was a better adhesive releasing agent needed by the shingle producer, but that he had to have it positioned precisely on the shingle wrapping material in order to have the adhesive strip on the top shingle coincide with the area treated with the adhesive releasing agent when shingles and wrapping material came together in the wrapping machine. What was required was the same order of precision as went into the positioning of the printing and other graphic material on the shingle wrapping paper and was felt necessary to an attractive and saleable packaging of the goods. The consequence

## 2

of this finding was the pursuit not only of a better adhesive releasing agent, but one which could be applied by a printing press when the graphics were imposed on the shingle wrapping paper. Another property which was sought for the adhesive releasing agent was a non-destructive or non-deleterious compatibility with the adhesive. It would not do to find a way of packaging the shingles cleanly and, nonetheless, to destroy their efficacy.

During trials, it was found that the shingle producer's latex emulsion would not print with good result. Several other materials were tried and found to print well, but they either released the adhesive on the shingles inadequately or attacked the adhesive's sealing properties. It was then found that a mixture of stearato chromic chloride (commercially available under the brand name "Quilon C"), water, and a neutralizer did the job well in all particulars. The adhesive releasing agent of such mixture which was imprinted on the inner side of kraft shingle wrappers over an area of about 4" x 40" per wrapper and at a rate of about 1.23 pounds of mixture per 1000 wrappers met the test of the shingle producer, i.e., gave complete release of the adhesive from a wrapper (without impairing the end use of the adhesive) after one week's exposure to 120° F. in a stack of eight bundles of twelve shingles per bundle.

Preferably, the mixture of the present invention consists of about 50% by weight of a concentrate of stearato chromic chloride in isopropyl alcohol having a solids content of about 27% to 30% by weight, about 47.5% by weight of water, and about 2.5% by weight of hexamethylene tetramine. It has been found that reducing the proportion of the concentrate to about 45% by weight causes the mixture to perform inadequately, but raising the proportion raises the mixture's cost without improving its performance. The ratio of concentrate to neutralizer should be about 20 to 1 at all times.

What is claimed is:

1. A printing method comprising formulating an adhesive releasing agent printable on paper at spaced intervals by means of a printing press which comprises a mixture of about 50% by weight of a concentrate of stearato chromic chloride in isopropyl alcohol having a solids content of about 27% to 30% by weight, about 47.5% by weight of water, and about 2.5% by weight of neutralizer and printing said agent on paper at spaced intervals by means of a printing press.
2. The method of claim 1 wherein the neutralizer is hexamethylene tetramine.

#### References Cited

##### UNITED STATES PATENTS

|           |         |         |       |         |
|-----------|---------|---------|-------|---------|
| 2,549,220 | 4/1951  | McLaren | ----- | 260—438 |
| 2,772,141 | 11/1956 | Dunlap  | ----- | 264—338 |
| 2,803,557 | 8/1957  | Martin  | ----- | 104—194 |

ALEXANDER H. BRODMERKEL, Primary Examiner.  
T. MORRIS, Assistant Examiner.